

Dec. 4, 1928.

1,694,258

R. C. HARTONG

PROCESS OF MANUFACTURING IMITATION LEATHER

Filed May 24, 1923



FIG. 1

FIG. 2



FIG. 3

INVENTOR

Robert C. Hartong

BY

R. D. Sibley

ATTORNEY

## UNITED STATES PATENT OFFICE.

ROBERT CLIFFORD HARTONG, OF AKRON, OHIO, ASSIGNOR TO SEIBERLING RUBBER COMPANY, OF AKRON, OHIO, A CORPORATION OF DELAWARE.

## PROCESS OF MANUFACTURING IMITATION LEATHER.

Application filed May 24, 1923. Serial No. 641,258.

My invention relates to imitation or artificial leather and the process of producing it, with the object in view of providing a serviceable article resembling leather, which shall have advantages over leather for many uses, and which may be supplied at a cost materially less than the cost of genuine leather.

With this end in view, my invention consists in coating a textile fabric, such as cotton sheeting, with a plastic water-proof material, but preferably with a rubber composition in the manner as hereinafter set forth, wherein a plurality of coats or layers of varying composition are applied by well known methods to a textile fabric and the rubber product vulcanized.

My invention further consists in an imitation leather possessing a very smooth, shiny surface, much resembling, but superior to the varnished (or lacquered) surface of patent leather, in that my product, being prepared of plastic and flexible materials, does not crack and break away from the surface during wearing as do the patent leather surfaces. It is possible, furthermore, to pass my material over embossing or graining rolls, and obtain a product carrying a raised or embossed surface, or one grained in imitation of grain leather.

It is also an object of my invention to produce a smooth, glossy surface on a textile fabric, friction-coated or impregnated with a compound of a plastic nature, by first applying the plasticized material or compound to a metallic liner and then removing the compound from the liner in a manner as herein-after set forth, whereby said liner transfers its own surface effects to the rubber composition attached thereto. This liner may be made of tin, aluminium, tinned-iron, or other surface treated iron, or may be an alloy, or in fact, any other metal or combination of metals, which do not form sulfides readily. It is, then, an object of my invention, to pro-

duce a product possessing a smooth, glossy surface by methods differing from those in common use, and to obtain this desirable and satisfactory surface appearance without the use of expensive molds, plates, hydraulic curving presses, or other cumbersome and expensive equipment in common use, thereby reducing the cost of equipment needed, and the amount of labor needed to manufacture the material.

In practicing this improved process, I pre-

pare a compound containing rubber and other ingredients, as set forth herein-after in detail, and then calender or coat this compound, which I will designate as "compound A" upon a metallic sheet, in the form of a metallic liner, by ordinary calendering practice. In order to give this "compound A" the proper backing, a textile, such as cotton sheeting, can be frictioned with a rubber-containing compound, hereinafter designated as "compound B". This textile containing "compound B", is then doubled upon "compound A", which, as was pointed out, has been previously calendered upon the metallic sheet or liner. By the term doubling, I refer to that process or step well known in the art of preparing a treated fabric whereby a fabric coated on one side with a layer of waterproof material is folded upon or laid against a second layer of waterproof material which in its turn may or may not have a fabric backing. That is two surfaces of waterproofing material, at least one of which has a suitable fabric backing, are folded or laid upon one another preferably by means of sufficient pressure usually applied by the calendering rolls to ensure a firm union between the waterproofing surfaces. This combination may then be tightly wrapped upon a cylindrical drum to the extent of several hundred yards in one continuous length, and the edges of the product tightly wrapped with curing aprons or wraps, as is commonly practiced in curing rubber sheet on drums, to protect the product from the bad effects of steam during the vulcanization process. When prepared in this manner, the product on the drum is cured in an ordinary open heat steam vulcanizer, or by any other well known method of curing rubber compounds by heat. After vulcanization, the product is unwrapped, and removed from the drum by means of any ordinary and well known method.

My preferred process of preparing the various compounds mentioned herein and my final product may be readily understood by reference to the drawings in which Figure 1 is a diagrammatic representation of a means of preparing the various compounds, Figure 2 is a diagrammatic representation of a means of preparing my final product and Figure 3 is a sectional view through the final product.

Referring to Figure 1, the rolls of a calen-

dering machine,  $R$ ,  $R^1$ ,  $R^2$ , are turning in the directions indicated by the arrows. Rubber or a suitable rubber composition 6, for example compound A, previously plasticized and 5 mixed on the differential rubber mills, is positioned as indicated before the two upper rolls,  $R$ ,  $R^1$ . A metallic liner 8, on a roll  $R^3$ , turning as indicated and guided by guide roll 9, is passed between rolls  $R^1$ ,  $R^2$  of the 10 calendering machine and has laid thereon a layer 7 of the rubber composition 6. The calendered product 10 comprising a metallic liner carrying on one side a composition hereinafter referred to as compound A, is then 15 wound upon roll  $R^4$ . Using the same equipment and the same process as just described but substituting a roll of textile fabric for the metallic liner before mentioned, the fabric may be coated with compound B. This coating 20 may be placed first on one side and then if desired, by reversing the roll of treated fabric and running it through the calendering machine as before described, a coating of the same or of a different composition may be 25 applied to the opposite side of the fabric.

Referring to Figure 2 of the drawings, a roll  $R^5$  carrying compound A calendered on the metallic liner and turning in the direction indicated, is doubled upon the compound 30 B calendered upon the fabric and positioned on roll  $R^3$  by passing the materials between the rolls  $R^1$ ,  $R^2$  of a calendering machine and winding the doubled product on the roll  $R^4$  as shown. This product may then be 35 wrapped and vulcanized in the manner as hereinafter described. As previously mentioned the metallic liner may be smooth or embossed with any design desired, and during the vulcanization process, the surface effects 40 of the liner are transferred to the rubber composition in contact therewith. After the vulcanization step is finished, the product is unwrapped and then unrolled and the metallic liner removed. The product is then ready 45 for use in any manner as desired.

This product, as shown in Figure 3, comprises a textile fabric 3, calendered upon one side with a plastic composition 2 (compound B) which is doubled upon another plastic 50 composition 1 (compound A), said textile fabric 3 being also calendered upon its opposite side with a plastic composition 4 (compound C), said composition 4 containing fibers as described. After buffing, a nap N 55 is raised over the surface of this compound. Inasmuch as the composition 1 (compound A) is preliminarily laid as described upon a metallic liner, the surface effects of the liner are transferred to the composition 1 to produce 60 an imitation patent leather surface S. In case the liner is embossed a similar effect is produced on the surface S.

Altho the nature of the rubber compound used is not an essential part of my invention, 65 the following composition is given as illus-

trative of one which serves very satisfactorily as the compound to be calendered on to the metallic liner, and referred to above as "compound A". For this compound, there are mixed on the differential mixing mills, 60 70 parts of rubber, 10 parts of gas black, 15 parts of sulfur, 10 parts of mineral rubber, 2 parts of the acetaldehyde derivatives of the polymerized ethylidene aniline (an accelerator known to the rubber trade as A-7),  $\frac{1}{2}$  part 75 of paraffin, 2 parts of cottonseed oil, and one part of "Cycline oil" (a compounded mixture of vegetable oil and mineral oil). "Compound B", which, as was mentioned above, is frictioned on the textile material, and then 80 doubled on "compound A", preferably has as its composition, 84 parts of rubber, 10 parts of glue,  $\frac{3}{4}$  parts of sulfur,  $\frac{1}{4}$  part of thiocarbanilid, 3 parts of cottonseed oil, and 2 parts of "Cycline oil". The methods of mixing 85 these materials, as well as variations in the quantities of, or even substitutions for, the ingredients themselves are apparent to those skilled in the art of rubber compounding. These formulæ are, however, illustrative of a type of compound that has proved 90 to be very successful in the practice of my invention. The time of cure necessary for vulcanizing these materials, varies according to the number of plies on the curing drum. For 95 example, a roll or drum, wrapped as described, and containing about 100 yards of my treated fabric, requires approximately 3 and  $\frac{1}{2}$  hours heating at 30 pounds steam pressure, with about 30 minutes additional in the heater 100 with the steam turned off to insure more uniform heat distribution.

The appearance and usefulness of the product prepared in the manner just disclosed, can be improved by calendering the textile material, preferably of cotton fabric, as was hereinbefore mentioned, on the side opposite the side carrying the "compound A". This calendering operation is done by the ordinary skim coating method of calendering, and consists 105 in simply spreading a thin film of a composition (referred to hereinafter as "compound C"), rendered plastic in the usual manner, onto a backing, preferably of fabric, or other equivalent material. The following rubber 110 composition is given as illustrative of the type I prefer to use for the calendering process just described. This composition, referred to in my description as "compound C", is prepared 115 in the usual manner, by breaking down, or plasticizing, on the differential rubber mixing rolls, 110 parts of rubber, preferably of the grade known as plantation rubber, and then adding and homogeneously incorporating therein, 135 parts of cotton linters, 20 120 parts of glue, 20 parts of zinc oxide, 70 parts of lithopone, 4 and  $\frac{1}{2}$  parts of sulfur, 2 parts of paraffin, 2 parts of phenanthrene,  $\frac{1}{2}$  part of cotton seed oil and  $\frac{1}{2}$  part of thiocarbanilid. The actual methods of mixing this 125 130

compound and of calendering it onto the cotton fabric, are so well known to those skilled in the art, that no further description of the actual process is necessary.

5 It is apparent, then, that I have prepared a product comprising a textile base, one side of which is skim-coated with "compound C", while the opposite side is friction-coated with "compound B", said "Compound B" being 10 doubled upon "Compound A", which has itself been previously calendered upon a metallic sheet or liner. The subsequent steps of finishing the product are the same as were mentioned before,—that is, the finished material is wrapped on a drum, the ends covered with curing aprons, and the product then cured in an open heat steam vulcanizer for the required period of time. After unwrapping the vulcanized product, the side carrying "compound C" is preferably buffed with emery cloth, carborundum cloth, or any abrasive material, or treated by any other process which will raise the nap in the "compound C". In this manner a surface is realized which 15 has all the appearance, as well as the necessary physical properties of, a suede leather. It is obvious, then, that this final product consists of a textile base, so treated with rubber compositions that one side has a smooth 20 glossy coating resembling patent leather, while the opposite side has a fibrous, nappy surface, resembling suede leather. This synthetic product has numerous advantages over all previously known artificial products of 25 the nature of leather.

The natural leather finish which is much to be desired in compounds of this type, can be even more closely imitated by using a metallic liner which can be embossed in the 30 well known manner upon an embossing calender. The process for making the product having an embossed surface is similar to the process already described, except that the metallic liner used has an embossed surface, 35 which transfers its surface effect to the rubber composition calendered thereon. The composition calendered is sufficiently stiff and firm to retain any markings impressed by the embossed liner, while pressure applied 40 in the wrapping on the drum for the vulcanizing step is not great enough to have any detrimental effect on the design transferred to the plastic composition. In order to obtain the best results, it is desirable, when 45 calendering "compound A" on this liner, to use an idler roll which is cloth covered. By means of this roll, pressure is applied to compound "A", after it has been calendered, so that it will flow properly into and thereby 50 completely fill the embossed surface of the metallic liner, in order to obtain a complete reproduction of the pattern desired. This embossed composition can now be used in 55 building up the artificial leather compound, according to the manner already described,—

that is, it has doubled upon it a textile base, friction coated with a compound "B", and the whole wrapped on a drum and cured.

Although the imitation patent leather finish, prepared by the process as set forth 70 is very durable, I have found that its wear-resisting qualities can be increased by a slight modification in the process. The textile base, already coated or calendered on one side with compound "B", may be ply-coated or calendered over this compound with a composition which I designate as compound "D", and which comprises 73 parts of rubber, 10 parts of glue, 4 parts of mineral rubber, 10 parts of gas black, 4 parts of refined uncured auto friction stock, 1 part of cotton seed oil, and  $\frac{3}{4}$  part of sulfur. The milling of this composition, and the calendering of it onto the textile base, are carried out by the usual methods. After compound 80 "C" has been applied to the opposite side of the fabric, and compound "A" has been doubled, in the manner as described, upon the side of the product carrying compounds "B" and "D", the product is vulcanized. In 90 this way I have prepared an artificial leather comprising a textile base, calendered on one side with compound "C", and on the opposite side with compound "B", together with a ply-coat of compound "D", which is then 95 doubled up on compound "A", previously calendered, and preferably, but not necessarily embossed upon the metallic liner. The whole is then vulcanized. By the use of this 100 ply stock of compound "D", interposed in my material between compound "B" and compound "A", the aging properties and resistance to cracking of compound "A" are very appreciably improved. This improvement is brought about by the employment of compound "D", which furnishes a tough and non-cracking under-coating or base for compound "A". Moreover, since compound "D" 105 contains such a small percentage of free sulfur, its use further improves compound "A", since there is probably a certain amount of sulfur migration from compound "A" into compound "D" during the vulcanization process. Since this migration would affect the aging properties of the material, this 110 would cause the inner portion of compound "A" to be more flexible, and noncracking than the outer portion, or the imitation patent leather surface. At the same time, use of this 115 ply-coated calendered compound "D", does not disturb the harder surface cure of compound "A", which gives to the material its characteristic leather like properties. Compound "A" has in itself, very high resistance 120 to cracking or to the effects of aging for the reason that while the degree of vulcanization is comparatively high, the flexibility of the product is maintained by the use of the combination of the oils used in the compound. Its desirable qualities are, however, further 125 130

enhanced by the use of the compound "D", applied as a ply coating over compound "B" as described.

Although in the examples set forth, I have specified the use of certain materials in certain proportions, it is to be understood that this is for purposes of illustration only and that my invention is limited solely by the claims appended hereto and made a part of this application and in which I intend to claim all novelty inherent in my invention which is permissible in view of the prior art.

What I claim is:—

1. A process of manufacturing an imitation leather, which comprises frictioning a plastic composition on a textile fabric, doubling said frictioned fabric upon a plastic composition previously calendered upon a metallic liner, and heat-treating the product.

2. A process of manufacturing an imitation leather, which comprises frictioning a rubber composition on a textile fabric, doubling said frictioned fabric upon a rubber composition previously calendered upon a metallic liner, and vulcanizing the product.

3. A process of manufacturing an imitation patent leather, which comprises calendering a rubber composition upon a smooth surface, capable of transferring its surface effects to said composition, doubling upon said composition a textile fabric frictioned with a rubber composition, and vulcanizing the product.

4. A process of manufacturing an imitation leather, which comprises frictioning a textile fabric on one side with a rubber composition, skim-coating said fabric on the side opposite said friction-coated side, with a rubber composition, doubling the friction coated side upon a rubber composition previously calendered upon a metallic liner, and vulcanizing the product.

5. A process of making an embossed imitation leather, which comprises friction-coating a textile fabric with a rubber composition, doubling said friction-coated fabric upon a rubber composition previously calendered upon an embossed metallic liner, and vulcanizing the product.

6. A method of producing a surface effect on a rubber composition, which comprises

calendering said rubber composition upon a metallic liner.

7. A method of producing a smooth surface effect on a plastic composition, which comprises calendering said plastic composition upon a metallic liner.

8. A method of producing an embossed surface on rubberized fabric, which consists in frictioning a rubber composition upon a textile fabric, doubling said frictioned fabric upon a rubber composition previously calendered upon an embossing calender, and vulcanizing the product.

9. An imitation leather comprising a textile fabric base, friction coated on both sides with a plastic composition, one side of said coated fabric being united to a rubber composition bearing an embossed surface, the opposite side of said coated fabric being united to a rubber composition carrying fibers.

10. An imitation patent leather comprising a textile fabric base, friction coated with a rubber composition, one side of said coated fabric being united to a rubber composition possessing a glossy surface.

11. An imitation leather comprising a foundation fabric friction coated on one side with a rubber composition containing fibers and friction coated on the opposite side with a second rubber composition having an embossed surface.

12. An imitation leather product consisting of rubber compositions applied to a fabric base, one side of said product being finished as an imitation patent leather, and the opposite side being finished as an imitation suede leather.

13. In the manufacture of an imitation leather, the process comprising calendering a textile fabric with a rubber composition, ply coating a rubber composition over said calendered fabric, calendering a rubber composition upon a metallic liner and doubling said compositions one upon the other.

14. An embossed imitation leather comprising a foundation fabric friction coated with a rubber-containing composition, said composition carrying a coating of a rubber composition having designs embossed thereon by an embossing calender.

ROBERT CLIFFORD HARTONG.